

3,706,595  
METHOD OF APPLYING A RESIN BINDER  
TO A SUBSTRATE

Arthur H. Drelich, Plainfield, and Bobby R. Bowman,  
East Brunswick, N.J., assignors to Johnson & Johnson  
No Drawing. Filed Jan. 22, 1971, Ser. No. 109,026  
Int. Cl. B44d 1/44; C08h 19/00

U.S. CL. 117—38

13 Claims

## ABSTRACT OF THE DISCLOSURE

Methods of controlling the migration of resin binders in the manufacture of bonded nonwoven fabrics from fibrous webs comprising the use of a resin binder composition comprising: (1) a synthetic resin; (2) a water soluble, polymeric, carboxylic thickener; and (3) a metal ammine, complex coordination compound capable of releasing ions of said metal to control the total migration of the resin binder during its deposition on the fibrous web.

The present invention relates to porous, absorbent fibrous sheet materials and to their methods of manufacture. More particularly, the present invention is concerned with the so-called bonded, "nonwoven" textile fabrics, i.e., fabrics produced from textile fibers without the use of conventional spinning, weaving, knitting or felting operations. Although not limited thereto, the invention is of primary importance in connection with nonwoven fabrics derived from "oriented" or carded fibrous webs composed of textile-length fibers, the major proportion of which are oriented predominantly in one direction.

Typical of such fabrics are the so-called "Masslinn" nonwoven fabrics, some of which are described in greater particularity in U.S. Patents 2,705,687 and 2,705,688, issued Apr. 5, 1955, to D.R. Petterson et al. and I. S. Ness et al., respectively.

Another aspect of the present invention is its application to nonwoven fabrics wherein the textile-length fibers were originally predominantly oriented in one direction but have been reorganized and rearranged in predetermined designs and patterns of fabric openings and fiber bundles. Typical of such latter fabrics are the so-called "Keybak" bundled nonwoven fabrics, some of which are described in particularity in U.S. Patents 2,862,251 and 3,033,721, issued Dec. 2, 1958 and May 8, 1962, respectively, to F. Kalwaites.

Still another aspect of the present invention is its application to nonwoven fabrics wherein the textile-length fibers are disposed at random by air-laying techniques and are not predominantly oriented in any one direction. Typical nonwoven fabrics made by such procedures are termed "isotropic" nonwoven fabrics and are described, for example, in U.S. Patents 2,676,363 and 2,676,364, issued Apr. 27, 1954, to C. H. Plummer et al.

And, still another aspect of the present invention is its application to nonwoven fabrics which comprise textile-length fibers and which are made basically by conventional or modified aqueous papermaking techniques such as are described in greater particularity in pending patent application Ser. No. 4,405, filed Jan. 20, 1970 by P. R. Glor and A. H. Drelich, and now abandoned. Such fabrics are also basically "isotropic" and generally have like properties in all directions.

The conventional base starting material for the majority of these nonwoven fabrics is usually a fibrous web comprising any of the common textile-length fibers, or mixtures thereof, the fibers varying in average length from approximately one-half inch to about two and one-half inches. Exemplary of such fibers are the natural fibers

such as cotton and wool and the synthetic or man-made cellulosic fibers, notably rayon or regenerated cellulose.

Other textile length fibers of a synthetic or man-made origin may be used in various proportions to replace either partially or perhaps even entirely the previously-named fibers. Such other fibers include: polyamide fibers such as nylon 6, nylon 66, nylon 610, etc.; polyester fibers such as "Dacron," "Fortrel" and "Kodel"; acrylic fibers such as "Acilan," "Orlon" and "Creslan"; modacrylic fibers such as "Verel" and "Dyne"; polyolefinic fibers derived from polyethylene and polypropylene; cellulose ester fibers such as "Arnel" and "Acele"; polyvinyl alcohol fibers; etc.

These textile length fibers may be replaced either partially or entirely by fibers having an average length of less than about one-half inch and down to about one-quarter inch. These fibers, or mixtures thereof, are customarily processed through any suitable textile machinery (e.g., a conventional cotton card, a "Rando-Webber," a papermaking machine, or other fibrous web producing apparatus) to form a web or sheet of loosely associated fibers, weighing from about 100 grains to about 2000 grains per square yard or even higher.

If desired, even shorter fibers, such as wood pulp fibers or cotton linters, may be used in varying proportions, even up to 100%, where such shorter length fibers can be handled and processed by available apparatus. Such shorter fibers have lengths less than  $\frac{1}{4}$  inch.

The resulting fibrous web or sheet, regardless of its method of production, is then subjected to at least one of several types of bonding operations to anchor the individual fibers together to form a self-sustaining web. One method is to impregnate the fibrous web over its entire surface area with various well-known bonding agents, such as natural or synthetic resins. Such over-all impregnation produces a nonwoven fabric of good longitudinal and cross strength, acceptable durability and washability, and satisfactory abrasion resistance. However, the nonwoven fabric tends to be somewhat stiff and boardlike, possessing more of the properties and characteristics of paper or board than those of a woven or knitted textile fabric. Consequently, although such over-all impregnated nonwoven fabrics are satisfactory for many uses, they are still basically unsatisfactory as general purpose textile fabrics.

Another well-known bonding method is to print the fibrous webs with intermittent or continuous straight or wavy lines, or areas of binder extending generally transversely or diagonally across the web and additionally, if desired, along the fibrous web. The resulting nonwoven fabric, as exemplified by a product disclosed in the Goldman Patent 2,039,312 and sold under the trademark "Masslinn," is far more satisfactory as a textile fabric than over-all impregnated webs in that the softness, drape and hand of the resulting nonwoven fabric more nearly approach those of a woven or knitted textile fabric.

The printing of the resin binder on these nonwoven webs is usually in the form of relatively narrow lines, or elongated rectangular, triangular or square areas, or annular, circular, or elliptical binder areas which are spaced apart a predetermined distance which, at its maximum, is preferably slightly less than the average fiber length of the fibers constituting the web. This is based on the theory that the individual fibers of the fibrous web should be bound together in as few places as possible.

The nominal surface coverage of such binder lines or areas will vary widely depending upon the precise properties and characteristics of softness, drape, hand and strength which are desired in the final bonded product. In practice, the nominal surface coverage can be designed so that it falls within the range of from about 10% to about 50% of the total surface of the final product. With-

in the more commercial aspects of the present invention, however, nominal surface coverages of from about 12% to about 40% are preferable.

Such bonding increases the strength of the nonwoven fabric and retains substantially complete freedom of movement for the individual fibers whereby the desirable softness, drape and hand are obtained. This spacing of the binder lines and areas has been accepted by the industry and it has been deemed necessarily so, if the stiff and board-like appearance, drape and hand of the over-all impregnated nonwoven fabrics are to be avoided.

The nonwoven fabrics bonded with such line and area binder patterns have had the desired softness, drape and hand and have not been undesirably stiff or board-like. However, such nonwoven fabrics have also possessed some disadvantages.

For example, the relatively narrow binder lines and relatively small binder areas of the applicator (usually an engraved print roll) which are laid down on the fibrous web possess specified physical dimensions and inter-spatial relationships as they are initially laid down. Unfortunately, after the binder is laid down on the wet fibrous web and before it hardens or becomes fixed in position, it tends to spread, diffuse or migrate whereby its physical dimensions are increased and its inter-spatial relationships decreased. And, at the same time, the binder concentration in the binder area is lowered and rendered less uniform by the migration of the binder into adjacent fibrous areas. One of the results of such migration is to make the surface coverage of the binder areas increase whereby the effect of the intermittent bonding approaches the effect of the over-all bonding. As a result, some of the desired softness, drape and hand are lost and some of the undesired properties of harshness, stiffness and boardiness are increased.

Various methods have been proposed to prevent or to at least limit such spreading, diffusing or migration tendencies of such intermittent binder techniques.

For example, U.S. Patent 3,009,822, issued Nov. 21, 1961 to A. H. Drelich et al., discloses the use of a non-migratory regenerated cellulose viscose binder which is applied in intermittent fashion to fibrous webs under the conditions wherein migration is low and the concentration of the binder in the binder area is as high as 35% by weight, based on the weight of the fibers in these binder areas. Such viscose binder possesses inherently reduced spreading, diffusing and migrating tendencies, thereby increasing the desired softness, drape and hand of the resulting nonwoven fabric. This viscose binder has found acceptance in the industry but the use of other more versatile binders has always been sought.

Resins, or polymers as they are often referred to herein as interchangeable terms, are high molecular weight organic compounds and, as used herein, are of a synthetic or man-made origin. These synthetic or manmade polymers have a chemical structure which usually can be represented by a regular repeating small unit, referred as a "mer," and are formed usually either by an addition or a condensation polymerization of one or more monomers. Examples of addition polymers are the polyvinyl chlorides, the polyvinyl acetates, the polyacrylic resins, the polyolefins, the synthetic rubbers, etc. Examples of condensation polymers are the pulurethanes, the polyamides, the polyesters, etc.

Of all the various techniques employed in carrying out polymerization reactions, emulsion polymerization is one of the most commonly used. Emulsion polymerized resins, notably polyvinyl chlorides, polyvinyl acetates, and polyacrylic resins, are widely used throughout many industries. Such resins are generally produced by emulsifying the monomers, stabilizing the monomer emulsion by the use of various surfactant systems, and then polymerizing the monomers in the emulsified state to form a stabilized resin polymer. The resin polymer is usually dispersed in an aqueous medium as discrete particles of colloidal dimensions (1 to 2 microns diameter or smaller) and is

generally termed throughout the industry as a "resin dispersion," or a "resin emulsion" or "latex."

Generally, however, the average particle size in the resin dispersion is in the range of about 0.1 micron (or 5 micrometer) diameter, with individual particles ranging up to 1 or 2 microns in diameter and occasionally up to as high as about 3 or 5 microns in size. The particle sizes of such colloidal resin dispersions vary a great deal, not only from one resin dispersion to another but even 10 within one resin dispersion itself.

The amount of resin binder solids in the resin colloidal aqueous dispersion varies from about  $\frac{1}{10}\%$  solids by weight up to about 60% by weight or even higher solids, generally dependent upon the nature of the monomers 15 used, the nature of the resulting polymer resin, the surfactant system employed, and the conditions under which the polymerization was carried out.

These resin colloidal dispersions, or resin emulsions, or latexes, may be anionic, non-ionic, or even polyionic 20 and stable dispersions are available commercially at pH's of from about 2 to about 11.

As will be pointed out in greater detail, such resin dispersions are used in the present inventive concept at alkaline pH ranges. Various alkaline reagents, such as 25 ammonia, are therefore added to bring the pH out of the acid range.

The amount of resin which is applied to the porous or absorbent material varies within relatively wide limits, depending upon the resin itself, the nature and character 30 of the porous or absorbent materials to which the resins are being applied, its intended use, etc. A general range of from about 4% by weight up to about 50% by weight, based on the weight of the porous or absorbent material, is satisfactory under substantially all uses. Within the 35 more commercial limits, however, a range of from about 10% to about 30% by weight, based on the weight of the porous or absorbent material, is preferred.

Such resins have found use in the coating industries for the coating of woven fabrics, paper and other materials. The resins are also used as adhesives for laminating materials or for bonding fibrous webs. These resins have also found wide use as additives in the manufacture of paper, the printing industry, the decorative printing of 40 textiles, and in other industries.

In most instances, the resin is colloidally dispersed in water and, when applied from the aqueous medium to a porous absorbent sheet material which contains additional water is carried by the water until the water is evaporated or otherwise driven off. If it is desired to place the resin 45 only on the surface of the wet porous or absorbent sheet material and not to have the resin penetrate into the porous or absorbent sheet material, such is usually not possible inasmuch as diffusion takes place between the aqueous colloidal resin and the water in the porous material. 50 In this way, the colloidal resin tends the spread into and throughout the porous material and does not remain merely on its surface.

Or, if it is desired to deposit the resin in a specific 55 intermittent print pattern, such as is used in bonding nonwoven fabrics, the aqueous colloid tends to diffuse and to wick along the individual fibers and to carry the resin with it beyond the confines of the nominal intermittent print pattern. As a result, although initially placed on the nonwoven fabric in a specific intermittent print pattern, the ultimate pattern goes far beyond that due to the spreading or migration which takes place due to the diffusion of the water and the resin, until the water is evaporated or otherwise driven off.

We have discovered new resin binder compositions containing polymers colloidally dispersed in aqueous media and new methods of applying such resin binder compositions to porous or absorbent fibrous materials, whereby the resins are applied in a controlled, relatively non-migrating manner. If it is desired that the resin be placed 60 only on the surface of the porous or absorbent material,

our compositions and methods will allow this to be done. Furthermore, if it is desired that the resin be impregnated throughout the material, from one surface to the other surface, again, our composition and method will allow this to be done.

We have now discovered an improved method of controllably depositing colloidal resin compositions on porous or absorbent materials whereby spreading, diffusing, and migration of the resin are controlled and are markedly reduced and wherein the concentration of the resin in the resin binder area reaches exceptionally high values in short distances as measured at right angles to the bond edge. When applied to fibrous webs in the manufacture of non-woven fabrics, excellent strength is obtained in the resulting bonded fabrics along with textile-like softness, 15 hand and drape.

The improved method involves the use of a resin dispersion which comprises from about 0.1% to about 60% by weight on a solids basis of a colloidal synthetic resin, from about 0.05% by weight to about 7% by weight, based on the weight of the colloidal synthetic resin solids of a water-soluble, polymeric, carboxylic thickener; and from about 0.01% by weight to about 5% by weight, based on the weight of the colloidal synthetic resin solids of a metal ammine complex coordination compound wherein the central metallic atom is chromium, nickel, zinc, or copper, said colloidal resin dispersion being stable at alkaline pH's in the presence of an excess of a complexing substance such as ammonium hydroxide and at certain concentrations or degrees of dilution but which is unstable at lesser concentrations or greater degrees of dilution when in the presence of heavy metal ions such as chromium, nickel, zinc, or copper.

The synthetic resin may be selected from a relatively large group of synthetic resins well known in industry for bonding purposes and may be of a self crosslinking type, externally cross-linking type, or not crosslinked. Specific examples of such synthetic resins include: Polymers and copolymers of vinyl ethers; vinyl halides such as plasticized and unplasticized polyvinyl chloride, polyvinyl chloride-polyvinyl acetate, ethylene-vinyl chloride, etc.; polymers and copolymers of vinyl esters such as plasticized and unplasticized polyvinyl acetate, ethylene-vinyl acetate, acrylic-vinyl acetate, etc.; polymers and copolymers of the polyacrylic resins such as ethyl acrylate, methyl acrylate, butyl acrylate, ethylbutyl acrylate, ethyl hexyl acrylate, hydroxyethyl acrylate, dimethyl amino ethyl acrylate, etc.; polymers and copolymers of the polymethacrylic resins such as methyl methacrylate, ethyl methacrylate, isopropyl methacrylate, butyl methacrylate, etc.; polymers and copolymers of acrylonitrile, methacrylonitrile, acrylamide, N-isopropyl acrylamide, N-methyloxy acrylamide, methacrylamide, etc.; vinylidene polymers and copolymers, such as polyvinylidene chloride, polyvinylidene chloride-vinyl chloride, polyvinylidene chloride-ethyl acrylate, polyvinylidene chloride-vinyl chloride-acrylonitrile, etc.; polymers and copolymers of polyolefinic resins including polyethylene, polypropylene, ethylene-vinyl chloride and ethylene-vinyl acetate which have been listed previously; the synthetic rubbers such as 1,2-butadiene, 1,3-butadiene, 2-ethyl-1,3-butadiene, high, medium and carboxylated butadiene-acrylonitrile, butadiene-styrene, chlorinated rubber, etc., natural latex; the polyurethanes; the polyamides; the polyesters; the polymers and copolymers of the styrenes including styrene, 2-methyl styrene, 3-methyl styrene, 4-methyl styrene, 4-ethyl styrene, 4-butyl styrene; natural latex; phenolic emulsions; etc.

These resins may be used either as homopolymers comprising a single repeating monomer unit, or they may be used as copolymers comprising two, three, or more different monomer units which are arranged in random fashion, or in a definite ordered alternating fashion, within the polymer chain. Also included within the inventive concept are the block polymers comprising relatively long 75

blocks of different monomer units in a polymer chain and graft polymers comprising chains of one monomer attached to the backbone of another polymer chain.

As pointed out previously, the compositions and formulations containing these polymers must be stable at an alkaline pH range of from about 7 to about 10½ or even higher which is the range wherein they are utilized, with preferred pH ranges extending from about 7½ to about 10. Such stability is particularly required for these polymer dispersions, when existing at their normal concentration levels in the presence of water-soluble polymeric carboxylic thickeners, and metal ammine complex coordination compounds, as described herein.

The water soluble polymeric carboxylic thickener may be selected from a relatively large group of such materials which include, for example: polyacrylic acid; polymeric crotonic acid; copolymers of vinyl acetate and crotonic acid; copolymers of vinyl acetate and acrylic acid; polyacrylic acid-polyacrylamide copolymers; polymethacrylic acid; polymethacrylic acid-polyacrylamide copolymers; carboxymethyl cellulose; carboxyethyl cellulose; carboxypropyl cellulose; polycarboxymethyl hydroxyethyl cellulose; alginic acid; polymers of acrylic acid and acrylic acid esters; polymers of  $\alpha,\beta$ -unsaturated carboxylic acids such as itaconic acid; etc. These water soluble, polymeric, carboxylic thickeners may be used in their acid forms but normally it is preferred to use their water soluble neutralized salts, that is, their sodium, potassium, lithium, ammonium, or like water soluble salts.

To the emulsion polymerized composition containing the colloidal resin is added a small amount of from about 0.01% by weight to about 5% by weight, based on the weight of the synthetic resin solids, of a metal ammine complex coordination compound wherein the central metallic atom is chromium, nickel, zinc, or copper.

Examples of metal ammine complex coordination compounds are:

hexammine chromium chloride



pentammine chloro chromium chloride



hexammine nickel chloride



hexammine nickel bromide



hexammine nickel chlorate



hexammine nickel iodide



hexammine nickel nitrate



tetrammine zinc carbonate



tetrammine zinc sulfate



diammine zinc chloride



tetrammine zinc chloride



diammine copper acetate



tetrammine copper sulfate



## tetrammine copper hydroxide



As defined herein, a metal ammine complex coordination compound is one of a number of types of metal complex compounds, usually made by addition of organic or inorganic atoms or groups such as ammonia ( $\text{NH}_3$ ) to simple inorganic compounds containing the metal atom. Coordination compounds are therefore essentially compounds to which atoms or groups are added beyond the number possible of explanation on the basis of electrovalent linkages, or the usual covalent linkages, wherein each of the two atoms linked donate one electron to form the duplet. In the case of the coordination compounds, the coordinated atoms or groups are linked to the atoms of the coordination compound, usually by coordinate valences, in which both the electrons in the bond are furnished by the linked atoms of the coordinated group.

The colloidal synthetic resin, the water soluble polymeric carboxylic thickener and the metal ammine complex coordination compound exist together in a stable emulsion form and normally do not agglomerate, coagulate or precipitate, as long as the stable concentration levels of  $\text{NH}_4\text{OH}$  or degree of dilution are maintained.

Subsequently, however, when the emulsion is diluted with water to a sufficiently low concentration of  $\text{NH}_4\text{OH}$ , the resin immediately coagulates and agglomerates in place with no further spreading, diffusion or migration.

It is believed that, when the emulsion is diluted sufficiently, the metal cation is released from the metal ammine complex coordination compound and immediately attacks or reacts with the water soluble polymeric carboxylic thickener causing the resin particles to agglomerate or coagulate.

It is also believed that the metal ammine complex coordination compound itself, as exemplified by tetrammine zinc chloride  $[\text{Zn}(\text{NH}_3)_4]\text{Cl}_2$ , ionizes to the divalent cation  $[\text{Zn}(\text{NH}_3)_4]^{++}$  and two anions  $\text{Cl}^-$ , even in the presence of high pH, ammoniacal, colloidal latex and water soluble, polymeric carboxylic thickener. Yet, this complex cation has no apparent or appreciable effect on the colloidal latex or on the water soluble, polymeric carboxylic thickener and specifically does not form an insoluble precipitate with either of them, as might have been expected.

As stated heretofore, it is further believed that dilution or otherwise diminishing the ammonium hydroxide content or concentration of the colloidal dispersion releases the  $\text{Zn}^{++}$  cation and this reacts with and insolubilizes the polymeric carboxylic thickener. Unexpectedly, however, the insolubilization of the polymeric carboxylic thickener also causes the colloidal latex itself to rapidly coagulate, even though the chemical reaction which takes place does not, insofar as is presently known, directly involve the latex, or its emulsifying or stabilizing system, if non-ionic.

Furthermore, methods have been discovered, as described herein to vary and control this unexpected sequence of chemical and physical events so as to controllably deposit a colloidal latex on the surface of, or in, or throughout a porous fibrous substrate. This method, as stated herein, can be used to very great advantage in print-bonding nonwoven fabrics or other porous substrates or in controllably placing and depositing latexes on a porous fibrous substrate or the like in the textile, paper, leather, and related industries.

It is also to be appreciated that, when the emulsion is diluted sufficiently, the metal cation which is released from the metal ammine complex coordination compound also is capable of attacking or reacting with any other chemical compounds which are present and which possess anionic groups, particularly hydroxy, carboxy, sulfino, sulfo, and like acid groups.

For example, the metal cation which is released immediately attacks a surfactant system which is anionic and contains surfactants such as alkyl aromatic sulfonic acids, alkyl sulfonic acids, the carboxylic acids, and other surfactants such as, for example, dodecyl

benzene sulfonate, octyl benzene sulfonate, hexyl benzene sulfonate, octadecyl benzene sulfonate, cetyl sulfonate, hexyl sulfonate, dodecyl sulfonate, octadecyl sulfonate, and the sodium and potassium fatty acid soaps containing from 5 to 18 carbon atoms. Other anionic surfactants include sodium p-1-methyl alkyl benzene sulfonates in which the alkyl group contains from 10 to 16 carbon atoms, the sodium di-n-alkyl sulfosuccinates in which the alkyl groups contain from 4 to 12 carbon atoms, the potassium n-alkyl malonates in which the alkyl group contains from 8 to 18 carbon atoms, the potassium alkyl tricarboxylates in which the alkyl group contains from 6 to 14 carbon atoms, the alkyl betaines in which the alkyl group contains from 6 to 14 carbon atoms, the ether alcohol sulfates, sodium n-alkyl sulfates, containing from 6 to 18 carbon atoms, etc.

The amount of surfactant used may vary from about 0.1% to 5% by weight of the resin solids dependent on the type resin being polymerized and the conditions under which it is polymerized.

The specific surfactant which is selected for use in the resin composition does not relate to the essence of the invention. It is merely necessary that it possess the necessary properties and characteristics to carry out its indicated function of stabilizing the resin composition prior to the time that coagulation and precipitation of the resin is required. Additionally, in the event that it is desired that the surfactant assist in or promote the coagulation and precipitation function, then it must possess the necessary anionic groups, as described hereinbefore, which are capable of reaction due to the presence of the metal cations released from the metal ammine complex coordination compound.

Moreover, the present inventive concept is operative with resins which have non-ionic or even polyionic emulsifying or stabilizing systems. The presence of an anionic surfactant system may be helpful in the controlled coagulation procedures described herein but it is not necessary or even especially advantageous in many cases.

The mechanism of instant agglomeration, coagulation and precipitation of the colloidal resin binder may therefore be triggered subsequent to dilution by reaction of the metal cation with either the water soluble, polymeric carboxylic thickener or the anionic surfactant, or both.

The dilution may be effected in different ways in order to activate the reaction mechanism. For example, the porous or absorbent fibrous material may be pre-treated by being pre-wet with a sufficient quantity of an aqueous medium, preferably water, whereby the colloidal resin composition immediately becomes sufficiently diluted. Or, if desired, the colloidal resin composition may be first printed on the porous or absorbent fibrous material and then substantially immediately treated with the aqueous medium such as water to effect the dilution whereupon the colloidal resin particles substantially immediately agglomerate or coagulate in place with no further spreading, diffusion or migration.

It is believed that the coagulation and precipitation take place by dilution alone wherein the  $\text{NH}_3$  groups in the metal ammine complex coordination compound break down and become  $\text{NH}_4\text{OH}$  in the excess water being carried by the fibrous web. By this reaction, the metal cations are released, coagulating and precipitating the resin. The reaction is believed to be as follows:



wherein Me is a metal such as disclosed herein, x is a whole number from 2 to 8 (and more commonly 2, 4 or 6), and Y is an anion such as chloride, iodide, bromide, sulfite, sulfate, nitrite, nitrate, carbonate, acetate, borate, phosphate, citrate, chlorate, oxalate, etc.

It is to be appreciated that Me and Y normally form compounds, the formation of which can be explained on the basis of electrovalent linkages, or the usual covalent

linkages, wherein each of the two atoms linked donate one electron to form the duplet.

It is believed that the addition of the water to the resin dispersion causes the equilibrium of the reaction mechanism to shift to the right whereby the metallic cations are released to bring about the described coagulation and precipitation of the resin. Lesser amounts of water cause the equilibrium of the reaction mechanism to move to the left favoring the continued stability of the metal ammine complex coordination compound and the resin dispersion.

The amount of the water applied to the fibrous web varies widely, depending upon many factors, the most important of which is the nature, concentration, properties and characteristics of the synthetic resin, the metal ammine complex coordination compound, and the surfactant system in which they are stabilized. Normally, the amount of water applied to the fibrous web is in the range of from about 140% to about 280%, and preferably from about 160% to about 220%, based on the weight of the fibrous web being treated. Such amounts are controlled by the use of suitable conventional vacuum apparatus, nip-rolls, squeeze-rolls, etc.

The amount of water which is applied to the fibrous web prior to the printing of the resin binder also affects the degree of control exercised over the coagulation and migration. The greater the amount of water, the greater is the control and the more rapid is the coagulation and the less is the migration. On the other hand, the less the amount of water in the fibrous web, the less is the control exercised, the less rapid is the coagulation, and the greater is the migration.

It is also to be realized that the greater the amount of water of dilution, then the greater is the degree of penetration of the resin binder into the fibrous web. And, the lesser the amount of water of dilution, then the lesser is the degree of penetration of the resin binder into the fibrous web.

The degree of coagulation may be lowered even more and the degree of migration may be increased by the inclusion in the pre-wetting water of a small amount of an alkaline or basic material such as ammonium hydroxide. The pH remains alkaline, just as it does in other variations of this invention, and the coagulation and precipitation are purely the result of the dilution.

When printed on a pre-wetted fibrous web during the manufacture of nonwoven fabrics, the total migration of the resin binder solids may be reduced to as little as about 50% or less beyond the originally deposited area. In some instances, the migration is relatively negligible. Normally, however, the increase in area of the resin binder solids, even under the most adverse conditions, does not materially exceed about 200%. Such values are to be compared to increases in binder migration of at least about 300% and up to about 800% when emulsion polymerized resins are applied to fibrous porous absorbent sheet materials, unaided by the principles disclosed herein.

The concentration of the binder resin solids in the binder area is correspondingly increased when utilizing the principles of the present invention and is in the range of from about 50% by weight to about 120% by weight, and more normally from about 60% to about 80% by weight, based on the weight of the fibers in the binder area.

The invention will be further illustrated in greater detail by the following specific examples. It should be understood, however, that although these examples may describe in particular detail some of the more specific features of the invention, they are given primarily for purposes of illustration and the invention in its broader aspects is not to be construed as limited thereto.

#### EXAMPLE I

A fibrous card web weighing about 570 grains per square yard and comprising 100% rayon fibers 1½ denier

and 1½ inches in length is intermittently print bonded by the rotogravure process using an engraved roll having 6 horizontal wavy lines per inch. The width of each line as measured on the engraved roll is 0.024 inch.

The composition by weight of the resin binder formulation used for the intermittent print-bonding is:

- (1) 7 lbs. of a 55% solids latex of Air Reduction Aircoflex 510, a copolymer of ethylene and vinyl acetate stabilized with a nonionic surfactant
- (2) 2 lbs. of water
- (3) 1 lb. of a 10% solution of a thickening agent, Rohm & Haas Acrysol 51, a copolymer of acrylic acid and acrylamide. Mol. wt. 375,000-500,000
- (4) 50 ml. of a 31% solution of zinc tetrammine chloride metal coordination complex (sp. gr. 1.13) containing 10% zinc equivalent or 17.5% zinc tetrammine chloride (actual).

The fibrous card web is pretreated or pre-moistened with a large amount of water to the extent of about 190% moisture based on the weight of the fibers in the web.

The extra dilution with water is sufficient by itself to upset the stability of the resin dispersion when applied to the web and it instantly coagulates and precipitates on the very wet fibrous web. The printed web is then processed, dried and cured.

The width of the binder line in the finished product is about 0.054 inch which represents a controlled total migration of about 125%. The surface coverage of the binder is about 32.4%. The percent binder in the bonded nonwoven fabric is about 17.4%. The concentration of binder in the binder area is about 54%, based on the weight of the fibers therein. Such measurements are obtained by procedures which are described in greater detail in copending patent application Ser. No. 65,880, filed Aug. 21, 1970.

The resulting nonwoven fabric has excellent strength, excellent softness, drape and hand, and excellent cross-resilience.

#### EXAMPLE II

The procedures of Example I are followed substantially as set forth therein with the exception that 160 grams of American Cyanamid curing resin Cyrez 933, an amino-

45 form melamine formaldehyde type external cross-linking agent, is added to the formulation. The results are good and are generally comparable to those obtained in Example I, except that this sample has improved wet-abrasion resistance and very good launderability. The resulting bonded nonwoven fabric also finds commercial acceptance.

#### EXAMPLE III

The procedures of Example II are followed substantially as set forth therein with the exception that the ethylene-vinyl acetate copolymer is replaced by 7 pounds of

55 46% solids latex of Goodrich 2671, a self cross-linking acrylic copolymer containing ethyl acrylate and acrylonitrile. The results are good and are generally comparable to those obtained in Example II. The resulting bonded nonwoven fabric also finds commercial acceptance.

#### EXAMPLE IV

65 The procedures of Example II are followed substantially as set forth therein with the exception that the ethylene-vinyl acetate copolymer is replaced by 7 pounds of a 55% solids latex of National Starch Resyn 2345, a copolymer of polyvinyl acetate and an acrylate containing 10% by weight of di-octyl phthalate plasticizer. The results are good and are generally comparable to those obtained in Example II except that this product has good wet-abrasion resistance and has very good launderability. The resulting bonded nonwoven fabric also finds commercial acceptance.

**11**  
**EXAMPLE V**

The procedures of Example I are followed substantially as set forth therein with the exception that the ethylene-vinyl acetate copolymer is replaced by 7 pounds of a 46% solids latex of Goodrich Geon 576, a plasticized polyvinyl chloride-lower alkyl acrylate copolymer stabilized with an anionic surfactant. The results are good and are generally comparable to those obtained in Example I except that this product has very good heat sealing properties. The resulting bonded nonwoven fabric also finds commercial acceptance.

**EXAMPLE VI**

The procedures of Example I are followed substantially as set forth therein with the exception that the ethylene-vinyl acetate copolymer is replaced by 7 pounds of a 50% solids latex of Rohm & Haas HA-8, a self cross-linking polyethyl acrylate copolymer stabilized with a non-ionic surfactant. The results are good and are generally comparable to those obtained in Example I. The resulting bonded nonwoven fabric also finds commercial acceptance particularly as a wet wiping cloth.

**EXAMPLE VII**

The procedures of Example II are followed substantially as set forth therein with the exception that the thickening agent is 1 pound of a 1% solution of the sodium salt of Hercules Carboxymethylcellulose 7H3S, having a high degree of polymerization in excess of about 1000, a high molecular weight in excess of about 200,000, a high viscosity of 900-3000 centipoises, maximum viscosity, 1% solution, at 25° C., and a degree of carboxymethyl substitution in the range of from about 0.65 to about 0.85 D.S. The results are good and are generally comparable to those obtained in Example II. The resulting bonded nonwoven fabric also finds commercial acceptance.

**EXAMPLE VIII**

The procedures of Example II are followed substantially as set forth therein with the exception that the thickening agent is 1 pound of a 9% solution of the sodium salt of Hercules Carboxymethylcellulose 7M, having a degree of polymerization in excess of 500, a medium molecular weight greater than about 70,000, a medium viscosity 30-100 centipoises, maximum viscosity, 1% solution, 25° C., and a degree of carboxymethyl substitution in the range of from about 0.65 to about 0.85 D.S. The results are good and are generally comparable to those obtained in Example II. The resulting bonded nonwoven fabric is also commercially acceptable.

**EXAMPLE IX**

The procedures of Example II are followed substantially as set forth therein with the exception that the thickening agent is 1 pound of a 9% solution of the sodium salt of Hercules Carboxymethylcellulose 12M8, having a medium molecular weight in excess of about 100,000, a medium viscosity of 400-800 centipoises, 2% solution, 25° C., and a degree of carboxymethyl substitution in the range of from about 1.2 to about 1.4 D.S. The results are good and are generally comparable to those obtained in Example II. The resulting bonded nonwoven fabric finds commercial acceptance.

**EXAMPLE X**

The procedures of Example IX are followed substantially as set forth therein with the exception that 1 pound of a 9% solution of the sodium salt of Hercules Carboxymethylcellulose 9M8 having a molecular weight of about 100,000 is used as the thickening agent. The results are good and are generally similar to those obtained in Example IX.

**12**  
**EXAMPLES XI AND XII**

The procedures of Example IX are followed substantially as set forth therein with the exception that the sodium salt of Hercules Carboxymethylcellulose 7M1 and 7H4 are used. 7M1 has a medium molecular weight, a medium carboxymethyl substitution of 0.65-0.85 D.S., and a low viscosity range in centipoises at 25° C. of 50-100 for a 2% concentration. 7H4 has a high molecular weight, a medium carboxymethyl substitution of 0.65-0.85 D.S., and a high viscosity range in centipoises at 25° C. of 2500-4500 for a 1% concentration. The results are good and are generally comparable to those obtained in Example IX. The resulting bonded nonwoven fabric is acceptable commercially.

**EXAMPLE XIII**

The procedures of Example II are followed substantially as set forth therein with the exception that the thickener is the sodium salt of Hercules Carboxymethylcellulose 7L2, having a low molecular weight of about 45,000, a degree of polymerization of about 200, a viscosity range in centipoises at 25° C. of 18 maximum at 2% concentration. An effect is noted but the results are not sufficient as to be commercially warranted.

**EXAMPLE XIV**

The procedures of Example II are followed substantially as set forth therein with the exception that the thickening agent is 1½ pounds of a 3% solution of the sodium salt of Hercules Carboxymethylcellulose 4M6, having a medium molecular weight of about 100,000, a medium viscosity, and a low degree of carboxymethyl substitution in the range of from about 0.38 to about 0.48 D.S. The results are good and are generally comparable to those obtained in Example II. The resulting bonded nonwoven fabric finds commercial acceptance.

**EXAMPLE XV**

The procedures of Example II are followed substantially as set forth therein with the exception that the thickening agent is 1 pound of a 10% solution of the sodium salt of Goodyear Carboset 514 polyacrylate copolymer. The results are good and are generally comparable to those set forth in Example II. The resulting bonded nonwoven fabric finds commercial acceptance.

**EXAMPLE XVI**

The procedures of Example II are followed substantially as set forth therein with the exception that the thickening agent is 1 pound of a 10% solution of a neutralized sodium salt of Rohm & Haas Acrysol A-5 polyacrylate homopolymer. The results are good and are generally comparable to those set forth in Example II. The resulting bonded nonwoven fabric finds commercial acceptance.

**EXAMPLE XVII**

The procedures of Example II are followed substantially as set forth therein with the exception that the thickener is 1 pound of a 5% solution of a sodium salt of Kelco Kelgin XL alginic water soluble, polymeric, carboxylic thickener. The results are good and are generally comparable to those obtained in Example II. The resulting bonded nonwoven fabric finds commercial acceptance.

**EXAMPLES XVIII AND XIX**

The procedures of Example II are followed substantially as set forth therein with the exception that the 50 milliliters of zinc tetrammine chloride is: (a) increased to 100 milliliters; and (b) decreased to 35 milliliters. The results in both cases are good and are generally comparable to those obtained in Example II. The resulting bonded nonwoven fabrics are commercially acceptable.

### 13 EXAMPLE XX

The procedures of Example II are followed substantially as set forth therein with the exception that the volume of zinc tetrammine chloride is increased from 50 milliliters to 100 milliliters and the amount of Acrysol 51 thickener is increased from 1 lb. to 1½ lbs. The results are good and are generally comparable to those obtained in Example II, except that it is noted that practically all of the resin binder is on one face of the nonwoven fabric whereby it may be more easily plied to another fabric or to another material.

EXAMPLES XXI AND XXII

The procedures of Example II are followed substantially as set forth therein with the exception that the zinc tetrammine chloride is replaced by an equivalent amount of: (a) zinc tetrammine sulfate; (b) zinc tetrammine carbonate; and (c) copper diammine acetate. The results in all three cases are good and are generally comparable to those obtained in Example II. The resulting bonded non-woven fabrics find commercial acceptance.

### EXAMPLE XXIII

The procedures of Example II are followed substantially as set forth therein with the exception that the water soluble polymeric carboxylated thickener is replaced by succinic acid which is a dicarboxylic acid. The results are not satisfactory and the use of succinic acid does not yield commercially acceptable products.

Having now described the invention in specific detail and exemplified the manner in which it may be carried into practice, it will be readily apparent to those skilled in the art that innumerable variations, applications, modifications, and extensions of the basic principles involved may be made without departing from its spirit and scope.

What is claimed is:

1. A method of applying a synthetic resin binder to a fibrous web of overlapping, intersecting fibers and controlling its migration thereon which comprises: applying to a fibrous web of overlapping, intersecting fibers a stable, colloidal aqueous dispersion having an alkaline pH comprising: (1) a synthetic resin; (2) a water-soluble, polymeric carboxylic synthetic resin; and (3) a metal amine complex coordination compound; and substantially immediately diluting said dispersion whereby a metal cation is released from said metal amine complex coordination compound to substantially immediately destroy the stability of said dispersion and coagulate said resin with a minimum of migration on said fibrous web.

2. A method as defined in claim 1 wherein the metal ammine complex coordination compound has the formula



wherein Me is a metal selected from the group consisting of chromium, nickel, zinc, and copper;  $x$  is a whole number from 2 to 8, inclusive; and Y is an anion.

3. A method as defined in claim 1 wherein the metal ammine complex coordination compound is zinc tetrammine sulfate.

4. A method as defined in claim 1 wherein the metal ammine complex coordination compound is zinc tetrammine carbonate.

5. A method as defined in claim 1 wherein the metal ammine complex coordination compound is zinc tetrammine chloride.

6. A method as defined in claim 1 wherein the metal ammine complex coordination compound is copper diamine acetate.

7. A method as defined in claim 1 wherein said aqueous dispersion comprises: from about 0.1% to about 60% by weight of said synthetic resin; from about 0.05% to about 7% by weight, based on the weight of said resin, of said water soluble, polymeric carboxylic thickening agent; and from about 0.01% to about 5% by weight, based on the weight of said resin, of said metal ammine complex co-ordination compound.

14

8. A method as defined in claim 1 wherein the dispersion is diluted with water.

9. A method of applying a synthetic resin binder to a fibrous web of overlapping, intersecting fibers and controlling its migration thereon which comprises: applying to a fibrous web of overlapping, intersecting fibers a stable, colloidal aqueous dispersion having an alkaline pH comprising: (1) a synthetic resin; (2) a water soluble, polymeric, carboxylic thickening agent; and (3) a metal ammine complex coordination compound, said dispersion being applied to said fibrous web in a predetermined, intermittent print pattern of spaced discrete areas; and substantially immediately diluting said aqueous dispersion whereby a metal cation is released from said metal ammine complex coordination compound to substantially immediately destroy the stability of said aqueous dispersion and to coagulate said synthetic resin in said spaced discrete areas with a minimum of migration therefrom.

10. A method of applying a synthetic resin binder to a fibrous web of overlapping, intersecting fibers and controlling its migration thereon which comprises: applying to a fibrous web of overlapping, intersecting fibers a stable, colloidal aqueous dispersion having an alkaline pH comprising: (1) a water-soluble, polymeric, carboxylic synthetic resin; and (2) a metal ammine complex coordination compound; and substantially immediately diluting said dispersion whereby a metal cation is released from said metal ammine complex coordination compound to substantially immediately destroy the stability of said dispersion and coagulate said resin with a minimum of migration on said fibrous web.

11. A method of applying a synthetic resin binder to a fibrous web of overlapping, intersecting fibers and controlling its migration thereon which comprises: applying to a fibrous web of overlapping, intersecting fibers a stable, colloidal aqueous dispersion having an alkaline pH comprising: (1) a water soluble, polymeric, carboxylic synthetic resin thickening agent; and (2) a metal ammine complex coordination compound, said dispersion being applied to said fibrous web in a predetermined, intermittent print pattern of spaced discrete areas; and substantially immediately diluting said aqueous dispersion whereby a metal cation is released from said metal ammine complex coordination compound to substantially immediately destroy the stability of said aqueous dispersion and to coagulate said synthetic resin in said spaced discrete areas with a minimum of migration therefrom.

12. A method of applying a stable resin composition to porous materials and controlling the migration thereon which comprises: applying to porous materials a stable resin composition having an alkaline pH and comprising: (1) a water-soluble, polymeric, carboxylic resin; and (2) a metal ammine complex coordination compound; and substantially immediately diluting said resin composition to substantially immediately destroy the stability of said resin composition and coagulate said resin whereby the migration of said resin on said porous materials is controlled.

13. A method of applying a stable resin composition to porous materials and controlling the migration thereon which comprises: applying to porous materials a stable resin composition having an alkaline pH and comprising: (1) a water-soluble, polymeric, carboxylic resin; (2) a metal ammine complex coordination compound; and (3) a synthetic resin; and substantially immediately diluting said resin composition to substantially immediately destroy the stability of said resin composition and coagulate said resins whereby the migration of said resins on said porous materials is controlled.

## References Cited

UNITED STATES PATENTS

- RE. 8,431 9/1878 Wheeler ----- 117-47  
1,979,121 10/1934 Rotta ----- 117-121

**15**

## UNITED STATES PATENTS

|           |         |                  |           |
|-----------|---------|------------------|-----------|
| 2,039,312 | 5/1936  | Goldman          | 117—140 X |
| 2,293,927 | 8/1942  | Beal             | 117—47    |
| 2,669,598 | 2/1954  | Marko et al.     | 117—47    |
| 2,676,363 | 4/1954  | Plummer et al.   | 117—140 X |
| 2,676,364 | 4/1954  | Plummer et al.   | 117—140 X |
| 2,705,687 | 4/1955  | Petterson et al. | 117—140 X |
| 2,705,688 | 4/1955  | Ness et al.      | 117—140 X |
| 2,862,251 | 12/1958 | Kalwaites        | 117—140 X |
| 2,880,114 | 3/1959  | Cohn et al.      | 117—47    |
| 2,943,955 | 7/1960  | Brill            | 117—121   |
| 2,971,934 | 2/1961  | Brown et al.     | 117—161 X |

10

**16**

|           |         |                |           |
|-----------|---------|----------------|-----------|
| 3,009,822 | 11/1961 | Drelich et al. | 117—161 X |
| 3,033,721 | 5/1962  | Kalwaites      | 117—140   |

## FOREIGN PATENTS

|   |         |         |        |         |
|---|---------|---------|--------|---------|
| 5 | 469,488 | 11/1950 | Canada | 117—121 |
|---|---------|---------|--------|---------|

WILLIAM D. MARTIN, Primary Examiner

M. R. P. PERRONE, JR., Assistant Examiner

U.S. CL. X.R.

|                                                     |
|-----------------------------------------------------|
| 117—44, 62, 121, 140 A, 161 R, 161 UC; 260—29.6 NR, |
| 29.6 RW                                             |